

## UNITED STATES PATENT OFFICE.

WILLOUGHBY STATHAM SMITH, OF BENCHAMS, NEWTON POPPLEFORD, AND HENRY JOSEPH GARNETT, OF SEVEN OAKS, ENGLAND.

## MAGNETIC ALLOY.

No Drawing. Original application filed January 10, 1924, Serial No. 685,432. Divided and this application filed May 2, 1925. Serial No. 27,593.

*To all whom it may concern:*

Be it known that we, WILLOUGHBY STATHAM SMITH, a subject of the King of Great Britain, residing at Benchams, Newton Poppleford, Devonshire, England, and HENRY JOSEPH GARNETT, a subject of the King of Great Britain, residing at Lymne, Solefields, Seven Oaks, Kent, England, have invented a new and useful Improvement in 10 Magnetic Alloys, of which the following is a specification.

This application is a division of our application Ser. No. 685,432, filed January 10, 1924.

15 This invention relates to the production of alloys possessing a high magnetic permeability especially at low magnetizing forces.

It is well known that it is desirable to add 20 inductance to telegraphic and telephonic cables and this has before been done by wrapping around the core of the cable an iron tape or wire.

Many research workers have been investigating the properties of various alloys, especially those of nickel and iron, with a view to discovering an alloy that should be suitable for this purpose. In our researches 25 we have found that an alloy may be made of nickel, copper and iron, which has a low hysteresis loss with a very high permeability at low magnetizing forces such as those present in telegraphic and telephonic cables.

According to our invention we make an 30 alloy of nickel, iron and copper, the nickel predominating, that is being at least 71% of the whole, while the iron is between 19 and 21% and copper between 5 and 6%.

In order also to increase the electrical 40 resistance of the alloy we preferably add to it a fourth element which may be tungsten, chromium, silicon, vanadium, titanium, molybdenum or aluminium; the amount of this fourth element is small compared to the amount of copper and is preferably less than 1%, since the addition of more than 1% of this fourth element, though increasing the resistance, will impair the permeability of the alloy considerably.

We also preferably include a small 50 amount of manganese to render the alloy more easy to forge.

The following are examples of alloys made in accordance with our invention

55

## No. 1.

An alloy consisting of:—

|           | Per cent. |    |
|-----------|-----------|----|
| Nickel    | 74.0      |    |
| Iron      | 20.0      | 60 |
| Copper    | 5.3       |    |
| Manganese | 0.7       |    |

has an initial magnetic permeability of 7000.

65

## No. 2.

An alloy consisting of:—

|           | Per cent. |    |
|-----------|-----------|----|
| Nickel    | 73.0      |    |
| Copper    | 5.4       | 70 |
| Iron      | 20.7      |    |
| Tungsten  | 0.6       |    |
| Manganese | 0.3       |    |

has an electrical resistance of 25 microhms per cubic centimetre and an initial magnetic 75 permeability of 6600.

## No. 3.

An alloy consisting of:—

|           | Per cent. |    |
|-----------|-----------|----|
| Nickel    | 73.0      | 80 |
| Copper    | 5.4       |    |
| Iron      | 20.7      |    |
| Silicon   | 0.6       |    |
| Manganese | 0.3       |    |

has an electrical resistance of 28 microhms per cubic centimetre and an initial magnetic 85 permeability of 5000.

## No. 4.

An alloy consisting of:—

|           | Per cent. |    |
|-----------|-----------|----|
| Nickel    | 73.0      |    |
| Copper    | 5.4       |    |
| Iron      | 20.5      | 95 |
| Vanadium  | 0.8       |    |
| Manganese | 0.3       |    |

has an electrical resistance of 31 microhms

per cubic centimetre and an initial magnetic permeability of 4700.

*No. 5.*

5 An alloy consisting of:—

|              | Per cent. |
|--------------|-----------|
| Nickel       | 72.5      |
| Copper       | 5.5       |
| Iron         | 21.0      |
| 10 Aluminium | 0.7       |
| Manganese    | 0.3       |

has an electrical resistance of 25.5 microhms per cubic centimetre and an initial magnetic permeability of 5500.

15 As has been said above, by increasing the amount of the fourth element the resistance may be further increased but the permeability may be considerably affected.

20 *No. 6.*

An alloy consisting of:—

|           | Per cent. |
|-----------|-----------|
| Nickel    | 72.6      |
| Copper    | 5.3       |
| 25 Iron   | 20.6      |
| Silicon   | 1.2       |
| Manganese | 0.3       |

has an electrical resistance of 32 microhms per cubic centimetre and an initial magnetic permeability of 3500.

These alloys are sensitive to heat-treatment and should be annealed by heating to a considerable temperature and then cooled.

35 This may conveniently be done by passing a wire or tape formed of the alloy through a tube heated electrically and allowing the wire or tape to cool rapidly as it issues from the tube.

40 If the correct temperature has not been used the magnetic properties will not be fully developed.

*Examples.*

45 Alloy No. 1, when heated to 600° C. and cooled in air, has an initial permeability of 800, when heated to 700° C. a permeability

of 2600, and when heated to 890° C. a permeability of 7000.

Moreover, when collectively annealed for 50 high initial permeability, the alloys have low hysteresis losses varying from 50 to 150 ergs per cubic centimetre with a maximum field of .25 c. g. s. units.

What we claim is:—

1. An alloy comprising nickel to the amount of at least 71%, iron to the amount of between 19% and 21% and copper to the amount of between 5% and 6%.

2. An alloy consisting of nickel 74%, iron 60 20%, copper 5.3% and manganese .7%.

3. An alloy consisting of nickel to the amount of at least 71%, iron to the amount of between 19% and 21%, copper to the amount of between 5% and 6% and a small 65 quantity of manganese.

4. An alloy comprising nickel to the amount of at least 71%, iron to the amount of between 19% and 21%, copper to the amount of between 5% and 6%, a small 70 quantity of manganese and tungsten.

5. An alloy comprising nickel to the amount of at least 71%, iron to the amount of between 19% and 21%, copper to the amount of between 5% and 6% and tungsten. 75

6. An alloy comprising nickel to the amount of at least 71%, iron to the amount of between 19% and 21%, copper to the amount of between 5% and 6% and a fourth 80 element adapted to increase the electrical resistance of the alloy.

7. An alloy comprising nickel to the amount of at least 71%, iron to the amount of between 19% and 21%, copper to the 85 amount of between 5% and 6%, another element adapted to increase the electrical resistance of the alloy and a small quantity of manganese.

In testimony that we claim the foregoing 90 as our invention we have signed our names this 21st day of April, 1925.

WILLOUGHBY STATHAM SMITH.  
HENRY JOSEPH GARNETT.